

Oct. 6, 1964

H. CHRISTENSEN ET AL  
EPITAXIAL DEPOSITION ON THE SURFACE  
OF A FRESHLY GROWN DENDRITE  
Filed May 25, 1962

3,152,022



INVENTORS: H. CHRISTENSEN  
R. S. WAGNER

BY *Stewart*

ATTORNEY

1

3,152,022

## EPITAXIAL DEPOSITION ON THE SURFACE OF A FRESHLY GROWN DENDRITE

Howard Christensen, Springfield, and Richard S. Wagner,  
Basking Ridge, N.J., assignors to Bell Telephone Laboratories, Incorporated, New York, N.Y., a corporation of New York

Filed May 25, 1962, Ser. No. 197,678  
3 Claims. (Cl. 148—175)

This invention concerns epitaxial deposition of semiconductors and, more particularly, epitaxial growth on semiconductor substrates prepared by dendritic growth.

Typical prior art techniques for the growth of epitaxial films on semiconductor substrates include elaborate and costly techniques for surface preparation preparatory to deposition. The usual slice cut from crystal ingot prepared in the ordinary fashion, such as by zone refining, possesses a surface which is unfit for epitaxial growth. The surface must first be lapped to remove the large surface discontinuities resulting from the cutting operation. This step may involve electromechanical or electrolytic polishing with or without mechanical abrading, the latter often involving a stepwise operation with abrasives of diminishing size. The surface is then washed, dried, and etched to remove strains introduced into the crystal surface during the abrading step. Another rinse follows with a final drying of the surface. All of these operations are time consuming and costly with the added danger of fracturing the crystal during abrading, or of incomplete or imperfect surface preparation ultimately resulting in a defective device unit.

These difficulties are overcome by the teachings of this invention. The invention consists essentially of preparing a semiconductor crystal by the technique of dendritic growth and, as a successive step in the same operation, depositing an epitaxial film on the freshly grown substrate.

A more thorough understanding of the invention may be obtained with the following detailed embodiment taken in conjunction with the drawing in which the figure is a schematic representation of an appropriate apparatus useful in carrying forth the principal operation of this invention.

The apparatus of the figure consists basically of a reaction chamber fitted for the introduction of the necessary gaseous components for the process and provided with appropriate heating means. The reaction vessel itself is a long vertical quartz tube 10 having approximate dimensions of 4 inches (diameter) by 3 feet (length). The tube contains a graphite crucible 11, filled with charge material for the melt from which the dendrite is pulled. Depending from the top of the tube is an electrically conductive pulling shaft 12, sealed with O-ring seal 13. The shaft terminates in a graphite tip 14 which serves as the seed holder. Surrounding the base portion of the quartz tube is an R.F. heating coil 15 contained in a container 16, for water-cooling the coil. An exhaust tube 17 is provided as shown.

The gas system here provides a means for evacuating the reaction chamber, flushing it with nitrogen and introducing a hydrogen atmosphere for pulling the crystal. Provision is made to alternatively direct the hydrogen through a source of semiconductor for the epitaxial deposition. In the system shown in the figure purified hydrogen and nitrogen are introduced at inlets 20 and 21 and into a flow meter 22. Valves 23 and 24 control the entry of the desired gas into the chamber. The single line 25 leaving the flow meter is divided into two separate paths the choice of which may be controlled by valves 26 and 27. The direct line leads into the reaction vessel through vacuum pump 28. The alternate portion of the

2

system is designed to provide a source material for epitaxial growth. The first stage of the epitaxy so system is a purifying operation which consists of passing the H<sub>2</sub> gas through tube 30 containing palladin 5 Alundum. The gas is then directed through a liquid nitrogen trap 31 which includes container 32 for liquid coolant. The purified gas leaving the trap is directed through the line 33 into the saturator 34 where the hydrogen is saturated with a semiconductor 10 compound. In this particular case the growth layer is to be germanium so that GeCl<sub>4</sub> is chosen as the source material contained in the saturator. The saturator is suspended in a cold bath 35 contained in beaker 36. cold bath is appropriately ethylene glycol and Dry 15 which maintains the GeCl<sub>4</sub> at -40° C. The inlet outlet to the saturator are controlled by valves 37 38. The outlet leads into the reaction vessel.

The heating circuit shown was used to provide the 1 necessary for the epitaxial deposition. It is connected 20 that the current flow is through the dendrite after the dendrite is pulled. For this purpose it is necessary 25 the dendrite not be withdrawn from the melt after 30 ing. The current flow from source 39 is adjusted so 25 the Joule heat in the dendrite maintains the proper 30 temperature for the epitaxial deposition. The conduct 35 crucible 11 and seed holder 14 are included for this 30 pose.

Other heating arrangements such as a tunnel furnace 30 are, of course, suitable. The latter has the advantage 35 of simple adaptability to continuous growth.

A specific operation using this apparatus is described 40 follows:

The system was flushed with nitrogen and a hydrogen atmosphere was introduced for the growth operation. 35 The crucible 11 was charged with 60 grams of high purity zone-refined germanium doped with arsenic to a resistivity of 1.3 ohm-cm. The seed crystal, the form of which 40 dictates whether the growth is polyhedral (slow) or dendritic (fast), necessarily contains at least two twin planes, for dendritic growth. The presence of a coherent twin plane presents a groove at the twin boundary along which nucleation and growth proceed rapidly. If only one twin plane is present the rapid growth is soon terminated because the ridges of the hexagonal platelet grow 45 at the expense of the grooves until the crystal is bounded wholly by ridges. Growth along a ridge is slow since it relies on surface nucleation and thus grows by polyhedral or slow growth. Two twin planes present a continuous available groove for continuous fast growth.

50 In this embodiment the seed crystal contained two twin planes parallel to (111) having external faces parallel to (111). The vertical direction (toward the melt) was [121]. The temperature of the melt, which is necessarily supercooled to a practical operating value by 55 least 3° C., was adjusted to give a stationary solid-liquid interface and then reduced about 10° C. as measured by a thermocouple 1/2 cm. below the surface. The crystal was then withdrawn at a rate of 0.5 cm./sec. The degree of supercooling bears a linear relation to the growth rate so that highly supercooled melts are preferred from a standpoint. A practical maximum in the degree of supercooling useful for this invention is 20° C.

60 The seed crystal may, of course, itself be a dendrite or it may be cut from a polyhedrally grown crystal. 65 In either case it must contain two twin planes. The size of the seed was approximately 5 cm. x 3 mm. x .1 in.

During the dendrite growth an atmosphere of hydrogen was maintained. The crystal was pulled to a length of about 20". The melt was allowed to solidify with the dendrite immersed. The heating circuit was turned 70 and the current through the dendrite was adjusted approximately 80 v. at 1 amp. The initial voltage

must be substantially higher due to the difference in resistivity encountered as the crystal heats. This power level was found to produce the desired deposition temperature, 835° C., as measured on an optical pyrometer. The hydrogen flow was diverted through the  $\text{GeCl}_4$  saturating system and adjusted to enter the chamber at 00 cc./min. The epitaxial deposition continued for ten minutes after which the heating circuit was disconnected and the gas flow returned to pure hydrogen. The dendrite was separated from the melt by using the R.F. heater to melt off the lower end. The system was flushed with nitrogen and the sample was removed.

The dendrite substrate has its long dimension in the (111) plane. The crystal was n-type as expected and had a resistivity of approximately 1.3 ohm-cm. The film obtained in the second or epitaxial growth step was examined by angle lapping and etching. It was found to be epitaxial in nature with a thickness of 8 microns. The film in this embodiment was also n-type. However, proper doping p-type films can also be obtained using the procedures of this invention.

As will be appreciated by those skilled in the art this invention is directed to epitaxial growth on a freshly prepared dendritically grown surface. Since this concept is more or less physical in nature it is obvious that it is applicable to any semiconductor material. While silicon and germanium are currently of primary practical interest, the III-V compounds are of increasing importance in semiconductor device development. III-V compounds of particular interest are GaAs, GaP and InSb. Epitaxial growths on dissimilar semiconducting substrates and particularly heterojunctions may also be grown according to the techniques of this invention. The conditions for epitaxial depositions according to this invention may be the same as those known in the art for deposition on linear polyhedrally grown semiconductor substrates. While the principles of dendritic growth are known in the art, the term is defined here as simply rapid crystal

growth, i.e., at least 0.01 cm./sec. from a supercooled melt on a seed crystal containing at least two parallel coherent twin planes. The growth occurs along a (111) crystal plane and may be of unlimited length. The latter fact suggests a continuous processing operation according to the present invention.

Various other modifications and extensions of this invention will become apparent to those skilled in the art. All such variations and deviations which basically rely on the teachings through which this invention has advanced the art are properly considered within the spirit and scope of this invention.

What is claimed is:

1. A method for growing an epitaxial semiconductor film on a semiconductor substrate which comprises suspending a seed crystal in a melt of the semiconductor desired as the substrate, said melt being supercooled at least 3° C., the seed crystal having at least two parallel twin planes, pulling the seed crystal from the melt at a rate of at least 0.01 cm./sec. in a direction parallel to the twin planes to form a dendrite and, as a successive step in the same process and in the same apparatus vapor-depositing an epitaxially grown semiconductor film on the surface of the freshly formed dendrite.
2. The method of claim 1 wherein the seed crystal has a diamond cubic crystal structure.
3. The method of claim 1 wherein the seed crystal has a zinc blende crystal structure.

#### References Cited in the file of this patent

#### UNITED STATES PATENTS

|           |         |                |
|-----------|---------|----------------|
| 2,854,363 | Seiler  | Sept. 30, 1958 |
| 3,031,403 | Bennett | Apr. 24, 1962  |

#### OTHER REFERENCES

"I.B.M. Technical Disclosure Bulletin," vol. 3, No. 2, July 1960, p. 45.